



US008034438B2

(12) **United States Patent**  
Sundstrom et al.

(10) **Patent No.:** US 8,034,438 B2  
(45) **Date of Patent:** Oct. 11, 2011

(54) **COATED CUTTING TOOL FOR GENERAL TURNING IN HEAT RESISTANT SUPER ALLOYS (HRSA)**

(75) Inventors: **Erik Sundstrom**, Fagersta (SE); **Rachid M'Saoubi**, Fagersta (SE); **Jon Andersson**, Fagersta (SE)

(73) Assignee: **Seco Tools AB**, Fagersta (SE)

(\*) Notice: Subject to any disclaimer, the term of this patent is extended or adjusted under 35 U.S.C. 154(b) by 364 days.

(21) Appl. No.: **12/195,578**

(22) Filed: **Aug. 21, 2008**

(65) **Prior Publication Data**

US 2009/0274899 A1 Nov. 5, 2009

(51) **Int. Cl.**

**B32B 9/00** (2006.01)

(52) **U.S. Cl.** ..... **428/216**; 51/307; 51/309; 428/336; 428/697; 428/698; 428/699

(58) **Field of Classification Search** ..... 51/307, 51/309; 428/216, 336, 697, 698, 699

See application file for complete search history.

(56) **References Cited**

U.S. PATENT DOCUMENTS

5,750,247 A \* 5/1998 Bryant et al. ..... 428/697  
6,214,287 B1 \* 4/2001 Waldenstrom ..... 75/240

6,273,930 B1 \* 8/2001 Waldenstrom ..... 75/240  
6,309,738 B1 \* 10/2001 Sakurai ..... 428/216  
6,612,787 B1 \* 9/2003 North et al. ..... 407/119  
6,884,497 B2 \* 4/2005 Sulin et al. ..... 428/216  
7,727,621 B2 \* 6/2010 Nordlof et al. ..... 428/699  
7,767,319 B2 \* 8/2010 Åkesson et al. ..... 428/697  
2003/0175536 A1 \* 9/2003 Penich et al. ..... 428/698  
2005/0129951 A1 \* 6/2005 Collin et al. ..... 428/336  
2007/0154739 A1 \* 7/2007 Martensson et al. ..... 428/698  
2008/0187775 A1 \* 8/2008 Ruppi et al. ..... 428/627

FOREIGN PATENT DOCUMENTS

|    |             |           |
|----|-------------|-----------|
| EP | 1 795 628   | 6/2007    |
| EP | 1 798 308   | 6/2007    |
| EP | 1 953 269   | 8/2008    |
| JP | 09-295204   | * 11/1997 |
| JP | 2003-127003 | * 5/2003  |
| JP | 2006-281363 | * 10/2006 |

\* cited by examiner

*Primary Examiner* — Archene Turner

(74) *Attorney, Agent, or Firm* — Young & Thompson

(57) **ABSTRACT**

The present invention relates to coated cemented carbide inserts, particularly useful in general turning of superalloys. The inserts are characterized by a cemented carbide of WC, about 5.0-7.0 wt-% Co, and about 0.22-0.43 wt-% Cr, where the substrate has a coercivity (Hc) of about 19-28 kA/m. The coating contains a single  $(\text{Ti}_x\text{Al}_{1-x})\text{N}$ -layer, where x is about 0.25-0.50, with crystal structure of NaCl type, total thickness of about 3.0-5.0  $\mu\text{m}$ , (200)-texture, and compressive residual strain of about  $2.5 \times 10^{-3}$ - $5.0 \times 10^{-3}$ , optionally containing an outermost TiN-layer.

**9 Claims, 1 Drawing Sheet**



**FIGURE 1**



1

**COATED CUTTING TOOL FOR GENERAL  
TURNING IN HEAT RESISTANT SUPER  
ALLOYS (HRSA)**

**CROSS REFERENCE TO RELATED  
APPLICATIONS**

This application claims priority to Swedish Application No. 0701910-2 filed Aug. 24, 2007, the entire disclosure of which is incorporated herein by reference.

**FIELD OF THE INVENTION**

The present invention relates to cutting tool inserts containing a cemented carbide substrate and a coating, particularly useful for general turning of heat resistant super alloys. Fine grained substrate in combination with a thick physical vapor deposition (PVD)-coating with a reduced residual strain level greatly improves the wear resistance.

**BACKGROUND OF THE INVENTION**

Superalloys are a broad range of nickel-, iron-, and cobalt-based alloys developed specifically for applications demanding exceptional mechanical and chemical properties at elevated temperatures. The classic use for these alloys is in the hot end of aircraft engines and land based turbines. Almost every metallurgical change made to improve the high temperature properties makes it more difficult to machine these alloys.

As high temperature strength is increased, the alloys become harder and stiffer at the cutting temperature. It results in increased cutting forces and increased wear on the cutting edge during machining.

Because stronger materials generate more heat during chip formation and because the thermal heat conductivity of these alloys is relatively low, very high cutting temperatures are generated, which also contributes to an increased wear of the cutting edge.

To make matters even worse, as the alloys are heat treated to modify the as-cast or solution treated properties, abrasive carbide precipitates or other second phase particles often form. These particles do also cause rapid wear of the cutting edge.

What is needed is a cutting tool insert containing coated cemented carbide, for general wet machining of superalloys, with improved wear resistance. The invention is directed to these, as well as other, important needs.

**SUMMARY OF THE INVENTION**

In one aspect, the invention is directed to cutting tool inserts, comprising a cemented carbide body and a coating particularly useful in general turning of superalloys, wherein the cemented carbide body comprises:

WC;

5.0-7.0, preferably 5.5-6.5, wt-% Co;

0.22-0.43, preferably 0.24-0.33, wt %-Cr; and

wherein the cemented carbide body has a coercivity,  $H_c$ , of about 19-28, preferably about 21-27, kA/m; and

wherein the coating comprises one layer of  $(Ti_xAl_{1-x})N$ ,

where  $x$  is about 0.25-0.50, preferably about 0.30-0.40 with a crystal structure of NaCl type and a total thickness of the layer of  $(Ti_xAl_{1-x})N$  of about 3.0-5.0  $\mu m$ , preferably about 3.5-4.5  $\mu m$ , measured on the middle of the flank face with a compressive residual strain of about  $2.5 \times 10^{-3}$ - $5.0 \times 10^{-3}$ , preferably about  $3.0 \times 10^{-3}$ - $4.0 \times 10^{-3}$  and with a texture coefficient  $TC(200)$  of about 1.6-2.1, the texture coefficient (TC) being defined as:

5

$$TC(hkl) = \frac{I(hkl)}{I_0(hkl)} \left[ \frac{1}{n} \sum_{n=1}^N \frac{I(hkl)}{I_0(hkl)} \right]^{-1}$$

where

10  $I(hkl)$ =intensity of the (hkl) reflection

$I_0(hkl)$ =standard intensity according to JCPDS card no 38-1420

N=number of reflections used in the calculation  
(hkl) reflections used are (111), (200), and (220).

15 In another aspect, the invention is directed to methods for making a cutting tool insert, comprising a cemented carbide body and a coating particularly useful in general turning of superalloys, comprising the steps of:

20 preparing a substrate by milling, pressing and sintering a composition comprising:

WC;

5.0-7.0, preferably 5.5-6.5 wt-% Co;

0.22-0.43, preferably 0.24-0.33, wt %-Cr; and

wherein said substrate has a coercivity,  $H_c$ , of about 19-28, preferably 21-27 kA/m; and

depositing a single layer of  $(Ti_xAl_{1-x})N$  on the substrate, where  $x$  is 0.25-0.50, preferably about 0.30-0.40, with a crystal structure of NaCl type and a total thickness of about

30 3.0-5.0  $\mu m$ , preferably about 3.5 and 4.5  $\mu m$ , measured on the middle of the flank face with a compressive residual strain of about  $2.5 \times 10^{-3}$ - $5.0 \times 10^{-3}$ , preferably about  $3.0 \times 10^{-3}$ - $4.0 \times 10^{-3}$  and with a texture coefficient  $TC(200)$  of about 1.6-2.1, the texture coefficient (TC) being defined as:

35

$$TC(hkl) = \frac{I(hkl)}{I_0(hkl)} \left[ \frac{1}{n} \sum_{n=1}^N \frac{I(hkl)}{I_0(hkl)} \right]^{-1}$$

where

40  $I(hkl)$ =intensity of the (hkl) reflection

$I_0(hkl)$ =standard intensity according to JCPDS card no 38-1420

n=number of reflections used in the calculation

(hkl) reflections used are: (111), (200), (220).

45 using arc evaporation of an alloyed, or Ti+Al composite cathode, wherein the cathode comprises about 25-50 at-% Ti, preferably 30 to 40 at-% Ti, and a current about 50-200 A depending on cathode size and cathode material, the substrate bias of about -20 V--35 V, a deposition temperature of about

50 400° C.-700° C. and grown in an Ar+N<sub>2</sub> atmosphere containing 0-50 vol-% Ar, preferably 0-20 vol-%, at a total pressure of 1.0 Pa to 7.0 Pa.

55 In yet other aspects, the invention is directed to methods for machining of a superalloy, comprising the step of:

using a cutting tool insert described herein.

**BRIEF DESCRIPTION OF THE DRAWINGS**

The accompanying drawings, which are included to provide a further understanding of the invention and are incorporated in and constitute a part of this specification, illustrate embodiments of the invention and together with the description serve to explain the principles of the invention. In the drawings:

FIG. 1 shows a fracture surface of a coated cemented carbide substrate according to the present invention in which:

1. Cemented carbide body and
2. Single layer of (Ti, Al)N.

#### DETAILED DESCRIPTION OF THE INVENTION

It has now surprisingly been found that a cemented carbide with low Co-content and submicron tungsten carbide (WC)-grain size coated with a single (Ti, Al)N-layer grown using physical vapor deposition greatly improves the productivity in general machining of superalloys under wet conditions.

According to the present invention there is now provided a coated cutting tool insert consisting of a substrate and a coating. The substrate contains tungsten carbide (WC), about 5.0-7.0, preferably about 5.5-6.5, most preferably about 5.8-6.2, wt-% Co, about 0.22-0.43, preferably about 0.24-0.33, most preferably about 0.26-0.29, wt-% Cr with a coercivity (Hc) of about 19-28, preferably about 21-27, preferably about 22.5-26.5 kA/m. Preferably, the edge radius of the inserts before coating is about 15-30  $\mu\text{m}$ .

The coating contains a single layer of  $(\text{Ti}_x\text{Al}_{1-x})\text{N}$ , where  $x$  is about 0.25-0.50, preferably about 0.30-0.40, most preferably about 0.33-0.35. The crystal structure of the (Ti, Al)N-layer is of NaCl type. The total thickness of the layer is about 3.0-5.0  $\mu\text{m}$ , preferably about 3.5-4.5  $\mu\text{m}$ . The thickness is measured on the middle of the flank face.

The layer is strongly textured in the (200)-direction, with a texture coefficient TC(200) of about 1.6-2.1.

The texture coefficient (TC) is defined as follows:

$$TC(hkl) = \frac{I(hkl)}{I_0(hkl)} \left[ \frac{1}{n} \sum_{n=1}^n \frac{I(hkl)}{I_0(hkl)} \right]^{-1}$$

where

$I(hkl)$ =intensity of the (hkl) reflection

$I_0(hkl)$ =standard intensity according to JCPDS card no 38-1420

$n$ =number of reflections used in the calculation

(hkl) reflections used are: (111), (200), and (220).

The layer is in compressive residual stress with a strain of about  $2.5 \times 10^{-3}$ - $5.0 \times 10^{-3}$ , preferably about  $3.0 \times 10^{-3}$ - $4.0 \times 10^{-3}$ .

On top of the (Ti, Al)N, a TiN-layer of a thickness of about 0.1-0.5  $\mu\text{m}$  may be deposited.

The present invention also relates to a method of making a coated cutting tool insert consisting of a substrate and a coating. The substrate is made by conventional powder metallurgical methods milling, pressing, and sintering. It has a composition comprising WC, about 5.0-7.0, preferably about 5.5-6.5, most preferably about 5.8-6.2, wt-% Co, about 0.22-0.43, preferably about 0.24-0.33, most preferably about 0.26-0.29, wt-% Cr with a coercivity (Hc) of about 19-28, preferably about 21-27, most preferably about 22.5-26.5, kA/m.

Before coating, the inserts are edge-honed by wet-blasting to an edge radius of preferably about 15-30  $\mu\text{m}$ .

The method used to grow the layer is based on arc evaporation of an alloyed, or composite cathode, under the following conditions: The Ti+Al cathode composition is about 25-50 atomic share (at-%) Ti, preferably about 30-40 at-% Ti, most preferably about 33-35 at-% Ti.

Before coating the surface is cleaned preferably by applying a soft ion etching. The ion etching is performed in an Ar atmosphere or in a mixture of Ar and H<sub>2</sub>.

The evaporation current is about 50-200 A, depending on cathode size and cathode material. When using cathodes of about 63 mm in diameter the evaporation current is preferably about 60-100 A. The substrate bias is about -20--35 V. The deposition temperature is about 400-700° C., preferably about 500-600° C.

The (Ti, Al)N-layer is grown in an Ar+N<sub>2</sub> atmosphere consisting of about 0-50 vol-% Ar, preferably about 0-20 vol-%, at a total pressure of about 1.0-7.0 Pa, preferably about 3.0-5.5 Pa.

On top of the (Ti, Al)N-layer a TiN-layer of about 0.1-0.5  $\mu\text{m}$  thickness may be deposited using Arc evaporation as known.

The present invention also relates to the use of inserts according to the above for wet machining of superalloys, such as Inconel 718, Inconel 625, Nimonic 81, Waspaloy or Ti6Al4V, at a cutting speed of about 20-75 m/min, a cutting depth about 0.2-2.5 mm and a feed of about 0.05-0.30 mm/rev.

Unless defined otherwise, all technical and scientific terms used herein have the same meaning as commonly understood by one of ordinary skill in the art to which this invention belongs. Although any methods and materials similar or equivalent to those described herein can be used in the practice or testing of the present invention, the preferred methods and materials are now described. All publications mentioned hereunder are incorporated herein by reference. Unless mentioned otherwise, the techniques employed or contemplated herein are standard methodologies well known to one of ordinary skill in the art. The materials, methods, and examples are illustrative only and not limiting.

The present invention is further defined in the following Examples, in which all parts and percentages are by weight and degrees are Celsius, unless otherwise stated. It should be understood that these examples, while indicating preferred embodiments of the invention, are given by way of illustration only. From the above discussion and these examples, one skilled in the art can ascertain the essential characteristics of this invention, and without departing from the spirit and scope thereof, can make various changes and modifications of the invention to adapt it to various usages and conditions.

#### Example 1

Cemented carbide cutting tool inserts of type CNMG120412-MR3 and CNMG120408-MF1 consisting of a substrate and a coating were prepared. The substrate was made by milling, pressing and sintering. The composition was 5.9 wt-% Co, 0.27 wt-% Cr and rest WC. The coercivity was 24.0 kA/m corresponding to an average WC grain size of about 0.80  $\mu\text{m}$ .

The inserts were wet-blasted to an edge-radius of 25  $\mu\text{m}$ .

The coating was grown using arc evaporation of a Ti<sub>0.34</sub>Al<sub>0.66</sub> cathode, 63 mm in diameter. The deposition was carried out in a 99.995% pure N<sub>2</sub> atmosphere at a total pressure of 4.5 Pa, using a substrate bias of -30 V for 60 minutes. The deposition temperature was about 530° C. The thickness of the layer was 3.8  $\mu\text{m}$  in the middle of the flank face. X-ray diffraction showed a strong (002)-texture with (TC)=1.8 and a residual strain of  $3.5 \times 10^{-3}$ .

FIG. 1 shows a fracture surface of the insert.

#### Example 2

CNMG120412-MR3 coated inserts from Example 1 were tested with regard to wear resistance in longitudinal medium-rough turning at the following conditions.

Work piece: Cylindrical bar  
 Material: Inconel 718  
 Cutting speed: 50 m/min  
 Feed: 0.25 mm/rev  
 Depth of cut: 2.0 mm  
 Remarks: Flood coolant  
 Reference: Seco CP200

## Results

The tool life criterion was the maximum time in cut in minutes at a cutting speed of 50 m/min giving a flank wear of 0.2 mm. The results are found in Table 1.

TABLE 1

| Grade      | Time in cut [min] |
|------------|-------------------|
| Invention  | 8.50              |
| Seco CP200 | 6.00              |

This test shows that the inserts according to the invention achieve about 40% longer tool life than Seco CP200.

## Example 3

CNMG120408-MF1 coated inserts from Example 1 were tested with regard to wear resistance in longitudinal fine turning at the conditions below.

Work piece: Cylindrical bar  
 Material: Inconel 718  
 Cutting speed: 55, 70 m/min  
 Feed: 0.15 mm/rev  
 Depth of cut: 0.5 mm  
 Remarks: Flood coolant  
 Reference: Seco CP200

## Results

The time in minutes to a flank wear of 0.2 mm was measured. The results are found in Table 2.

TABLE 2

| Cutting speed           | 55        | 70           |
|-------------------------|-----------|--------------|
| Invention<br>Seco CP200 | —<br>7.00 | 7.00<br>5.00 |

This test shows that the inserts according to the invention increase tool life productivity by 40% compared to Seco CP200.

## Example 4

CNMG120412-MR3 coated inserts from Example 1 were tested with regard to tool life in a medium-rough boring operation at the conditions below.

Work piece: Special component  
 Material: Inconel 718  
 Cutting speed: 37 m/min  
 Feed: 0.20 mm/rev  
 Depth of cut: 3.2 mm  
 Remarks: Flood coolant  
 Reference: Competitor grade

## Results

Reference grade machined reached full tool life after 7 minutes and 40 seconds. The inserts according to the invention reached full tool life after 11 minutes and 50 seconds.

This test shows that the inserts according to the invention increase tool life up to 50%.

When ranges are used herein for physical properties, such as molecular weight, or chemical properties, such as chemical formulae, all combinations and subcombinations of ranges specific embodiments therein are intended to be included.

The disclosures of each patent, patent application, and publication cited or described in this document are hereby incorporated herein by reference, in their entirety.

Those skilled in the art will appreciate that numerous changes and modifications can be made to the preferred embodiments of the invention and that such changes and modifications can be made without departing from the spirit of the invention. It is, therefore, intended that the appended claims cover all such equivalent variations as fall within the true spirit and scope of the invention.

What is claimed is:

1. A cutting tool insert, comprising:  
 a cemented carbide body; and  
 a coating,

wherein the cemented carbide body comprises:

WC;  
 5.0-7.0 wt-% Co;  
 0.22-0.43 wt %-Cr; and  
 wherein the cemented carbide body has a coercivity,  $H_c$ , of about 19-28 kA/m; and  
 wherein the coating comprises one layer of  $(Ti_xAl_{1-x})N$ , where  $x$  is about 0.25-0.50, with a crystal structure of NaCl type and a total thickness of the layer of  $(Ti_xAl_{1-x})N$  of about 3.0-5.0  $\mu m$ , measured on the middle of the flank face with a compressive residual strain of about  $2.5 \times 10^{-3}$  and  $5.0 \times 10^{-3}$ , and with a texture coefficient  $TC(200)$  of about 1.6-2.1, the texture coefficient (TC) being defined as:

$$TC(hkl) = \frac{I(hkl)}{I_0(hkl)} \left[ \frac{1}{n} \sum_{n=1}^n \frac{I(hkl)}{I_0(hkl)} \right]^{-1}$$

where

$I(hkl)$ =intensity of the  $(hk\bar{l})$  reflection

$I_0(hkl)$ =standard intensity according to JCPDS card no 38-1420

$N$ =number of reflections used in the calculation

$(hk\bar{l})$  reflections used are: (111), (200), and (220).

2. A cutting tool insert according to claim 1, wherein the composition comprises about 5.5-6.5 wt-% Co.

3. A cutting tool insert according to claim 1, wherein the composition comprises about 0.24-0.33 wt %-Cr.

4. A cutting tool insert according to claim 1, wherein the composition has a coercivity,  $H_c$ , of about 21-27 kA/m.

5. A cutting tool insert according to claim 1, wherein  $x$  is about 0.30-0.40.

6. A cutting tool insert according to claim 1, wherein the total thickness of the layer of  $(Ti_xAl_{1-x})N$  is about 3.5-4.5  $\mu m$ .

7. A cutting tool insert according to claim 1, wherein the compressive residual strain is about  $3.0 \times 10^{-3}$ - $4.0 \times 10^{-3}$ .

8. A cutting tool insert according to claim 1, wherein the outermost TiN-layer has a thickness of about 0.1-0.5  $\mu m$ .

9. A cutting tool insert according to claim 1, wherein the cutting tool insert has an edge radius of about 15-30  $\mu m$  before coating.

\* \* \* \* \*